

## UNITED STATES PATENT OFFICE

CARL PIERCE LEWIS, OF BURLINGAME, CALIFORNIA, ASSIGNOR TO MINERALS SEPARA-TION NORTH AMERICAN CORPORATION, OF NEW YORK, N. Y., A CORPORATION OF MARYLAND.

## CONCENTRATION OF ORES.

No Drawing.

Application filed March 31, 1924. Serial No. 703,260.

To all whom it may concern:

Be it known that I, CARL PIERCE LEWIS, a citizen of the United States, and a resident of Burlingame, county of San Mateo, State 5 of California, have invented certain new and useful Improvements in Concentration of Ores, of which the following is a specification.

This invention relates to the froth-flotation concentration of ores, and is herein described as applied to the froth-flotation of certain ores with the aid of certain organic compounds containing sulphur. It has been found that the froth-flotation process is carried out much more efficiently when there are present in the ore pulp certain of the sulphur derivatives of carbonic acid such as those that yield anions and cations in solution. According to the present invention 20 the froth-flotation process is carried out with the aid of a sulphur derivative of carbonic acid in an acid ore pulp, the requisite acidity being usually obtained through the presence of sulphuric acid in the pulp.

25 The amount of acid used may vary widely. Sometimes, in the case of an ore containing acid-soluble mineral enough has been used to dissolve a large proportion of the acid-soluble mineral, with the result that the resulting metal-bearing pulp liquid carries it away. This may be precipitated, if desired, as is well known. Often, however, by a careful adjustment of conditions much less acid can be used.

30 For laboratory purposes potassium xanthate was prepared as follows:

198.4 grams of 88.5% caustic potash was dissolved in 524 grams ethyl alcohol (denatured #5 formula) at a temperature of 40 124° F., in a reflux condenser. The solution was cooled to 58° F. It contained a large excess of alcohol over the theoretical amount needed for the subsequent reactions. To this was added, while stirring, and in a 45 cooling bath, the theoretical amount of carbon disulphide. The reaction was substantially instantaneous, producing a thick pulp of potassium xanthate. The pulp was cooled and centrifuged in a laboratory machine, 50 yielding crystals containing about 20% moisture. The yield thus obtained was 74.7%. Another 17.5% was obtained by evaporation of the mother liquor. Both the centrifuged crystals and the residue from

the mother liquor gave excellent results in 55 flotation. It was found in cases where sulphuric acid was used according to the present invention that the centrifuged material yielded better results than the uncentrifuged. It has also been found that 60 excellent results can be obtained by using, instead of a pure or ordinary xanthate, the product obtained when concentrated alcoholic potash is mixed one-third its volume 65 of pine oil and there is obtained a precipitate by adding CS<sub>2</sub> in an amount somewhat in excess of that needed to combine with the ethyl alcohol present.

In one test a pulp of Anaconda slimes was agitated with sulphuric acid at the rate of 70 25 pounds per ton, and the pine-oil-xanthate complex mixture at the rate of 0.4 pound per ton. The results are shown in the following table:

|            | % Wt. | % Assays cu. | % Recoveries cu. |
|------------|-------|--------------|------------------|
| Heads..... | 100.0 | 2.83         |                  |
| Conc.....  | 31.9  | 8.64         | 97.1             |
| Tails..... | 68.1  | .12          | 2.9              |

75

80

Sometimes it has been found advantageous to preagitate the pulp with xanthate, and then add the acid. Good results were obtained with 5 pounds of sulphuric acid 85 added in this way to a pulp of Anaconda slimes.

In one regular run covering five hours at the rate of 120 tons per day of fresh Anaconda slimes, xanthate was added at the 90 head of the machine, 0.4 pound per ton. The other reagents used were a mixture of hardwood creosote and kerosene acid sludge, 5.0 pounds, and sulphuric acid, 20 pounds per ton. The tails contained 0.15% sulphide copper and 0.23% acid soluble copper, making a total of 0.38% recovered copper 95 against a normal of 0.61% recovered in the absence of xanthate.

During a seven and one-half hours run 100 on current Anaconda slimes at the rate of one hundred and eleven tons per twenty-four hours in a minerals separation standard machine, from a feed containing 3.28% copper, 0.26% being acid soluble copper, there was recovered a concentrate containing 11.43% cu. and 36.9% insolubles, the latter being a proportion desirable for 105

smelting. The tailings contained 0.29% copper of which 0.20% was acid soluble copper. This test was run at a temperature of 82° F. using for reagents, 7.89 pounds of 5 kerosene acid sludge, 21.6 pounds of chamber sulphuric acid, 2.36 pounds of hardwood creosote, and 2.92 pounds of a twenty per cent. solution of potassium xanthate in water, all quantities being in pounds per 10 short ton of ore.

Anaconda old gravity concentration tailings reground for flotation were treated at the rate of four hundred and eleven tons per twenty-four hours in a minerals separation standard machine provided with a porous bottom in the spitzkasten through which air was admitted. From a feed containing 0.52% copper, of which 0.12% was acid soluble copper, there was recovered a 20 concentrate containing 5.72% copper and 48% insolubles. The tailings from this contained 0.13% copper of which 0.08% was acid soluble. This test was run at a temperature of 50° F., using for reagents; 25 per ton of solids, 0.67 pounds of a 30% solution of potassium xanthate in water, 3.96 pounds of kerosene acid sludge, and 11.45 pounds of chamber sulphuric acid.

Having thus described certain embodiments of the invention what is claimed is:

1. The process of concentrating ores which consists in agitating a suitable acid pulp

of an ore with a mineral-frothing agent and a sulphur derivative of carbonic acid yielding anions and cations in solution to produce by the action of both a mineral-bearing froth containing a large proportion of a mineral of the ore, and separating the froth.

2. The process of concentrating ores which consists in agitating a suitable acid pulp of an ore with a mineral-frothing agent and a xanthate to produce by the action of both a mineral-bearing froth containing a large proportion of a mineral of the ore, and separating the froth.

3. The process of concentrating ores which consists in agitating a suitable pulp of an ore with a mineral-frothing agent and a xanthate and sulphuric acid to produce by the action of both a mineral-bearing froth containing a large proportion of a mineral of the ore, and separating the froth.

4. The process of concentrating ores which consists in agitating a suitable pulp of an ore with a mineral-frothing agent and a sulphur derivative of carbonic acid yielding anions and cations in solution and sulphuric acid to produce by the action of both a mineral-bearing froth containing a large proportion of a mineral of the ore, and separating the froth.

In testimony whereof, I have affixed my signature to this specification.

CARL PIERCE LEWIS.